

Patented Nov. 7, 1922.

1,434,642

UNITED STATES PATENT OFFICE.

CLIFFORD A. WOODBURY, OF MEDIA, PENNSYLVANIA, ASSIGNOR TO E. I. DU PONT DE NEMOURS & COMPANY, OF WILMINGTON, DELAWARE, A CORPORATION OF DELAWARE,

NITROGLYCERINE EXPLOSIVE.

No Drawing.

Application filed March 9, 1920. Serial No. 364,396.

To all whom it may concern:

Be it known that I, CLIFFORD A. WOODBURY, a citizen of the United States, and a resident of Media, in the county of Delaware and State of Pennsylvania, have invented 5 certain new and useful Nitroglycerine Explosives, of which the following is a specification.

My invention relates to nitroglycerine explosives and comprises explosives of this kind containing ammonium perchlorate.

Dynamites containing nitroglycerine, through continued use over a long period of time, have become recognized as standards 15 in the dynamite industry and in spite of the many new explosives developed, have maintained their leadership. Among the several reasons for this, the most important is undoubtedly the surety of action inherent in 20 a nitroglycerine dynamite. This surety is brought about through the sensitiveness of the nitroglycerine which is such as to be little altered by factors which tend to lower sensitiveness. Dynamites not containing 25 nitroglycerine are at best inclined to be rather insensitive to detonation by means of blasting caps, and are easily rendered too insensitive for practical use by influences which have no serious effect on nitroglycerine 30 dynamites.

Dynamites containing nitroglycerine, though of extended use, have always had certain undesirable properties. Among these, the more important are high sensitiveness, 35 to shock, ease of ignition, and tendency to exude nitroglycerine particularly in the case of high strength explosives where a high percentage of nitroglycerine must be used. Furthermore, with high strength nitro- 40 glycerine dynamites it is impracticable to supply the necessary oxygen for the combustible absorbent on account of the high percentage of absorbent that has to be used in order to properly hold all of the nitro- 45 glycerine. This leads to the production of noxious gases on explosion, thus seriously affecting the use of such explosive in under- ground work.

Glycerine, from which nitroglycerine is 50 made, is obtained as a by-product in the manufacture of soap, and the quantities produced are very limited in comparison with the demand for explosives using nitro- glycerine.

Many efforts have been made to find sub-

stitutes for nitroglycerine in dynamites and the most successful have been along the lines of utilizing ammonium nitrate to replace a portion of the nitroglycerine. Such explosives are much safer than straight nitro- 60 glycerine dynamites due to being much less sensitive to shock and far more difficult to ignite. On the other hand, ammonium nitrate explosives are extremely hygroscopic, 65 absorbing moisture so rapidly that they become unfit for use when stored for any appreciable length of time in humid climates. Furthermore, due to the peculiar habit of ammonium nitrate to change its crystalline form at about 90° F., such explosives have 70 a great tendency to set extremely hard when stored in climates where the temperature at times reaches or exceeds 90° F.

I have discovered that the substitution of ammonium perchlorate for a portion of the 75 nitroglycerine in dynamites containing nitro- glycerine results in explosives much less inflammable and less sensitive to shock, but still retaining in a large measure the surety of detonation and propagation and the low 80 hygroscopicity inherent in straight nitro- glycerine dynamites. In other words, the substitution of ammonium perchlorate for a portion of the nitroglycerine improves the 85 explosive from the point of view of safety 90 in a manner similar to improvement obtained by using ammonium nitrate, without introducing such undesirable properties as excessive hygroscopicity and tendency to set hard during storage. Furthermore, it is 95 practicable to replace a much greater proportion of nitroglycerine when using ammonium perchlorate than is the case when using ammonium nitrate, due to the fact that the former does not decrease the sensitiveness to detonation and propagation to nearly so great an extent as is true with the latter.

For example, I have found that an explosive containing 10 parts of nitroglycerine and 30 parts of ammonium perchlorate ex- 100hibits an ability to propagate detonation almost exactly equal to that exhibited by an explosive containing 20 parts of nitro- glycerine and 28 parts of ammonium nitrate.

Another important feature of my invention is that by substituting ammonium perchlorate for a portion of the nitro- glycerine there can be produced high grade 110 nitroglycerine dynamites free from a tend.

ency to exude nitroglycerine and so balanced as to oxygen content as to give unobjectionable gases on explosion. In underground work involving the blasting of hard rock, 5 explosives of the so-called gelatine type are used almost to the exclusion of all other types. These explosives are comprised of nitroglycerine gelatinized with a small percentage of nitrocotton and absorbed or 10 mixed with various materials such as alkali-metal nitrates, non-explosive absorbents, for example wood pulp, etc. Under present circumstances there is a rather low limit to the percentage of nitroglycerine which can be 15 used in such explosives and still retain a favorable oxygen balance, due to the high percentage of carbonaceous material, such as wood pulp, which has to be used in order to avoid exudation of the nitroglycerine. A 20 portion of the nitroglycerine can, it is true, be replaced by ammonium nitrate and a proper oxygen balance of the explosive itself thereby obtained; but this introduces another complicating factor, for, due to the 25 hygroscopicity of the nitrate of ammonia, it is necessary to give further protection to the explosive by coating it with an extra quantity of water-proofing material such as paraffine, and, inasmuch as the paraffine 30 is consumed in the explosion, the oxygen balance of the explosive is thereby upset, with the result that excessive quantities of carbon monoxide are formed. On account of the low hygroscopicity of ammonium 35 perchlorate, it is not necessary to use an extra amount of paraffine, thereby making possible the manufacture of high grade gelatine dynamites of the proper oxygen balance for underground work.

40 Examples of gelatine dynamites with and without ammonium perchlorate are:

### I.

|                   |             |
|-------------------|-------------|
| Nitroglycerine    | 70.0        |
| Nitrocotton       | 2.6         |
| Sodium nitrate    | 16.4        |
| Wood pulp         | 10.0        |
| Chalk             | 1.0         |
| <b>Total</b>      | <b>100.</b> |
| Oxygen deficiency | 5.12        |

### II.

|                       |             |
|-----------------------|-------------|
| Nitroglycerine        | 40.0        |
| Nitrocotton           | 0.8         |
| Ammonium perchlorate  | 30.00       |
| Sodium nitrate        | 18.2        |
| Carbonaceous material | 10.0        |
| Chalk                 | 1.0         |
| <b>Total</b>          | <b>100.</b> |
| Oxygen excess         | 7.12        |

(that is, the proportion of oxygen above 45 that required to combine with all the car-

bon and hydrogen present to form  $\text{CO}_2$  and  $\text{H}_2\text{O}$ .)

Though I have described the use of ammonium perchlorate in nitroglycerine explosives, I do not wish to confine myself to 70 explosives in which the liquid explosive ingredient is comprised solely of this material. As a matter of fact, I prefer to use liquids 75 composed of nitroglycerine in which is dissolved other compounds useful for depressing or retarding the freezing of the nitroglycerine, for example, aromatic nitro compounds, nitrated sugars, nitrated polymerized glycerine, etc. The nitrated polymerized glycerine is nitrated diglycerol; both the 80 nitrated sugar and the nitrated polymerized glycerol may therefore be referred to as a nitrate of an aliphatic compound having at least 6 and at most 12 carbon atoms and at least 4 hydroxy groups. 85

As typical examples of these new explosives I give the following:

|                                | III. | IV.  | V.   | VI.  | VII.  | VIII. | 90  |
|--------------------------------|------|------|------|------|-------|-------|-----|
| Nitroglycerine                 | 10   | 8    | 6.5  | 40   | 32    | 28    |     |
| Nitrated sugar                 |      |      | 1.5  |      |       |       | 4   |
| Nitro aromatic (TNT)           |      | 2    | 2    |      |       | 8     | 8   |
| Ammonium perchlorate           | 30   | 30   | 30   | 27   | 27    | 27    |     |
| Sodium nitrate                 | 41   | 42   | 43   | 20   | 22    | 20    |     |
| Carbonaceous material          | 18   | 17   | 16   | 12   | 10    | 12    |     |
| Chalk                          | 1    | 1    | 1    | 1    | 1     | 1     | 95  |
|                                | IX.  | X.   | XI.  | XII. | XIII. | XIV.  |     |
| Nitroglycerine                 | 25   | 20   | 18   | 25   | 20    | 18    |     |
| Nitrated polymerized glycerine |      | 5    | 4    |      | 5     | 4     | 100 |
| Nitro aromatics                |      |      | 3    |      |       | 3     |     |
| Nitrocotton                    | 0.6  | 0.6  | 0.6  | 0.6  | 0.6   | 0.6   |     |
| Ammonium perchlorate           | 30   | 30   | 30   | 10   | 10    | 10    |     |
| Sodium nitrate                 | 22   | 22   | 24   | 48   | 48    | 48    |     |
| Carbonaceous combustible       | 21.4 | 21.4 | 19.4 | 15.4 | 15.4  | 15.4  |     |
| Chalk                          | 1    | 1    | 1    | 1    | 1     | 1     |     |

105 The above examples illustrate the wide range of proportions in which the several ingredients may be used. In general I consider it desirable to have nitroglycerine present to the extent of at least 5%, and to have 110 ammonium perchlorate present in the proportions of from about 10 to 35%, based on the total weight of the dynamite. The proportion of carbonaceous material which I prefer lies between 8 and 25%, and that of the alkali metal nitrate, between 15 and 45%. Although from 10 to 35% of ammonium perchlorate will ordinarily be sufficient, a much greater proportion, for instance up to 65%, 115 may be used upon occasion.

120 I claim:

1. A dynamite comprising nitroglycerine, from about 10 to 35% of ammonium perchlorate, and a carbonaceous combustible material.

2. A dynamite comprising from 6.5 to 40% of nitroglycerine, from about 10 to 35% of ammonium perchlorate, and a carbonaceous combustible material.

3. A dynamite comprising at least 5 parts 125

of nitroglycerine, from about 10 to 35 parts of ammonium perchlorate, and from about 8 to 25 parts of a carbonaceous combustible material.

- 5 4. A dynamite comprising from 6.5 to 40 parts of nitroglycerine, from about 10 to 35 parts of ammonium perchlorate, and from about 8 to 25 parts of a carbonaceous material.
- 10 5. An explosive comprising from about 5 to 50 parts of nitroglycerine and from about 10 to 35 parts of ammonium perchlorate.
6. A nitroglycerine dynamite containing a sufficient amount of ammonium perchlorate 15 to render the oxygen content of the dynamite greater than that required to combine with all the carbon and hydrogen present to form  $\text{CO}_2$  and  $\text{H}_2\text{O}$ .
7. An explosive comprising nitroglycerine, 20 in which a nitrate of an aliphatic compound having at least 6 and at most 12 carbon atoms and at least 4 hydroxy groups is dissolved, ammonium perchlorate and a carbonaceous, non-explosive material.
- 25 8. An explosive comprising at least 5% of nitroglycerine, in which a nitrate of an aliphatic compound having at least 6 and at most 12 carbon atoms and at least 4 hydroxy groups is dissolved, ammonium perchlorate, 30 an alkali-metal nitrate, and a carbonaceous, non-explosive material.
9. An explosive comprising from 6.5 to 40 parts of nitroglycerine, in which a nitrate of an aliphatic compound having at least 6 and at most 12 carbon atoms and at least 4 hydroxy groups is dissolved, from about 10 to 35 parts of ammonium perchlorate an al-

kali-metal nitrate, and from about 8 to 25 parts of a carbonaceous, non-explosive material.

10. An explosive comprising nitroglycerine, in which nitrated polymerized glycerine is dissolved, ammonium perchlorate, and a carbonaceous non-explosive material.

11. An explosive comprising at least 5% of nitroglycerine, in which nitrated polymerized glycerine is dissolved, ammonium perchlorate, an alkali-metal nitrate, and a carbonaceous, non-explosive material.

12. An explosive comprising from 6.5 to 50 40 parts of nitroglycerine, in which nitrated polymerized glycerine is dissolved, from about 10 to 35 parts of ammonium perchlorate, from about 15 to 45 parts of an alkali-metal nitrate, and from about 8 to 35 parts 55 of a carbonaceous, non-explosive material.

13. An explosive comprising nitroglycerine, nitrated polymerized glycerine, ammonium perchlorate, an alkali-metal nitrate, and a carbonaceous, non-explosive material.

14. A dynamite comprising at least 5% of nitroglycerine, from about 10 to 35% of ammonium perchlorate, from about 15 to 45% of an alkali-metal nitrate, a carbonaceous non-explosive material, and a nitrate of an 65 aliphatic compound having at least 6 and at most 12 carbon atoms and at least 4 hydroxy groups.

15. A dynamite of the composition set forth in claim 14 and containing from 6.5 to 70 40% of nitroglycerine.

In testimony whereof I affix my signature.

CLIFFORD A. WOODBURY.

#### Certificate of Correction.

It is hereby certified that in Letters Patent No. 1,434,642, granted November 7, 1922, upon the application of Clifford A. Woodbury, of Media, Pennsylvania, for an improvement in "Nitroglycerine Explosives," errors appear in the printed specification requiring correction as follows: Page 3, line 26, claim 8, for the misspelled word "notroglycerine" read *nitroglycerine*, and line 55, claim 12, for the number "85" read 95; and that the said Letters Patent should be read with these corrections therein that the same may conform to the record of the case in the Patent Office.

Signed and sealed this 8th day of January, A. D., 1923.

[SEAL.]

KARL FENNING,

*Acting Commissioner of Patents.*